

## 1

3,165,862

## MULCH PAPER

Rex S. Harper, Mobile, and Curtis A. Gentry, Chickasaw, Ala., assignors to International Paper Company, New York, N.Y., a corporation of New York  
No Drawing. Filed Dec. 11, 1962, Ser. No. 243,720  
5 Claims. (Cl. 47—9)

This invention relates to the formation of a non-woven fabric from wood pulp fibers. More particularly, it relates to the production of a new material, from wood pulp fibers and without the use of water, for plant mulching.

It is known to use wood pulp fibers in, for instance, plant mulching and in such a manner that a non-woven fabric made of such fibers is laid down. See U.S. Patent No. 3,017,720, issued January 23, 1962, and copending U.S. application Serial No. 167,925, filed January 22, 1962. But, in such instances, large quantities of water are employed and the laying down, which is done at the plant site, requires mixers, pumps, hoses, spray heads of a size, number, and complexity such that it is largely inconceivable that any individual home owner or even country club manager can afford or will wish to encumber himself with them.

A way has now been found, however, for using wood pulp fibers as a plant mulch and otherwise which is, literally, within the grasp of such individuals. It involves the formation by manufacturers of sheets or rolls of non-woven groundwood or chemical, e.g., sulfate or sulfite, wood pulp fibers in the absence of water and binding agents and the, if desired, manual placement of such sheets or blankets over fertilized or unfertilized grass, flower, or other seed beds by individuals, preparatory to a simple wetting down with a garden hose or the like to achieve a mulch covering or superior protective and growth enhancing properties.

Broadly, in accordance with the present invention, wood pulp fibers are subjected to a three step process. First, the fibers are flash dried to reduce their moisture content to, preferably, about 5 to 25%, based on the bone dry weight of the fibers. Next, the fibers are formed into a mat in the absence of water and binding agents on commercially available equipment. Then, the mat is substantially finished for use by the homeowner or the like by subjection to pressure and, preferably, heat under, for example, standard calender rolls adapted to deliver about 300 to 2000 lbs. pressure per lineal inch and a surface temperature in the range of about 200 to 400° F.

More specifically, and by way of example, baled, flash dried sulfate pulp—which has, desirably, been dyed green both for aesthetic reasons and as a deterrent to attack by birds and the like once it has been put to its ultimate use—is delivered to a hammermill such as the commercially available pre-opener made by Curlator Corporation. There, the bales are broken up and the fibers are fluffed. Next, the fluffed fibers which are about  $\frac{1}{4}$  inch or less in length are conveyed by pneumatic or mechanical means, but without water or binding agents, to another Curlator machine, the 60-B Special Rando-Feeder and Rando-Webber. The fiber travels through such machine—the essential elements of which are a first suction roll or so-called condenser for forming a precursor mat of fibers, a doctoring device for removing the precursor mat from the condenser, a lickerin for breaking up the precursor mat

## 2

and assuring a more even fiber distribution in the subsequent re-matting, and a second condenser for forming the desired mat—and emerges as a blanket or fabric having a thickness of from about  $\frac{1}{2}$  to  $1\frac{1}{2}$  inches. The blanket is then travelled to a calender stack wherein a patterned steel roll adapted to be heated and a felted or rubber roll are positioned to deliver a nip pressure of about 500 lbs. per lineal inch and a surface temperature of about 300° F. to the blanket. An embossing calender of 66 inch length which is made commercially by B. F. Perkins and Sons, Inc. has been used for this purpose and, with it, there have been produced blankets ranging in density from 3.3 to 6.2 ounces per square yard or 200 to 400 lbs. per 1,000 square yards and having sufficient bursting strength as measured by the Mullen test to permit satisfactory handling, i.e., slitting to desired widths, winding into rolls, wrapping, transportation to seedbed sites, and un-rolling over such sites.

Thus far, the blankets of the present invention have been given even greater strength by compressing together several plies thereof at elevated pressures, e.g., 5000 lbs. per lineal inch or by bubbling steam therethrough. Presumably, this could also be done by adding binding agents during the mat formation and activating such agents at the pressure or calendering station. The uses of the products of such steps are clearly many. Backing sheets for resins and foams, insulation in drinking cups or structural panels, wrapping and packaging materials, fiberboard, wall board, insulating board, and outdoor protective coverings for machines, building materials and fuels, just-poured concrete, and many others come to mind. Indeed, the whole range of uses for the products of a tree including paper and paperboard made on a Fourdrinier machine and lumber, plywood, and veneers cannot be excluded at this time.

However, more immediately, it has already been found that a blanket of the present invention made from sulfate wood pulp fibers of  $\frac{1}{4}$  inch or less in length and having a density of about 4.97 ounces per square yard or 310 lbs. per 1,000 square yards produces surprisingly superior results when employed as a plant mulch with a rate of application of about 1,000 to 1,500 lbs. per acre. When applied to the soil, and there thoroughly wetted, the blanket appears to disintegrate to form a cellulosic fiber to soil particle bond. The intimate contact with the surface soil particles results, it is believed, in a porous mat which allows young seedlings from newly germinated plants to penetrate the cover. This is in sharp contrast to the situation where the cover stems from a wet process in situ paper sheet formation and holds together as a membrane, so as to deny intimate association of cellulosic fiber and soil particle and free passage to seedlings. And, the end result is that, in, for instance, grass establishment, the blanket of the present invention yields thicker and more uniform grass growth than any wet-formed product.

What is claimed is:

1. A process consisting essentially of forming flash dried wood pulp fibers selected from the group consisting of groundwood and chemical wood pulp fibers into a mat by suction means and embossing the mat at a pressure in the range of about 300 to 2,000 lbs. per lineal inch.
2. A process consisting essentially of forming flash dried sulfate wood pulp fibers having a length of about  $\frac{1}{4}$  inch into a mat by suction means and embossing the mat

at a pressure of about 500 lbs. per lineal inch and at a temperature of about 300° F.

3. The process of claim 1 wherein the embossing is conducted at a temperature in the range of about 200° F. to 400° F.

4. A mulching product consisting essentially of an embossed blanket of flash dried wood pulp fibers selected from the group consisting of groundwood and chemical wood pulp fibers, the blanket having a density of about 200 to 400 lbs. per 1,000 square yards.

5. A mulching product consisting essentially of an embossed blanket of flash dried sulfate wood pulp fibers having a length of about  $\frac{1}{4}$  inch, the blanket having a density about 310 lbs. per 1,000 square yards.

References Cited by the Examiner

UNITED STATES PATENTS

|    |           |       |                |       |           |
|----|-----------|-------|----------------|-------|-----------|
|    | 1,625,066 | 4/27  | Viersen        | ----- | 18—47.5   |
|    | 1,931,248 | 10/33 | Bryant         | ----- | 47—9      |
| 5  | 1,978,102 | 10/34 | Clapp          | ----- | 47—1      |
|    | 2,215,244 | 9/40  | Linzell        | ----- | 162—206 X |
|    | 2,348,081 | 5/44  | Linzell        | ----- | 18—47.5   |
|    | 2,489,079 | 11/49 | Clark et al.   | ----- | 19—155 X  |
| 10 | 2,925,360 | 2/60  | Roberts et al. | ----- | 19—156    |
|    | 3,129,466 | 4/64  | L'Hommedieu    | ----- | 19—161 X  |

ABRAHAM G. STONE, Primary Examiner.

T. GRAHAM CRAVER, Examiner.